

March 21, 1933.

J. A. YUNKER

1,902,747

PROCESS OF RE-FORMING NATURAL GAS

Filed July 8, 1930



Inventor:

James A. Yunker,

By *Byers, Townsend & Trotter,*  
Attorneys.

## UNITED STATES PATENT OFFICE

JAMES A. YUNKER, OF LOUISVILLE, KENTUCKY, ASSIGNOR TO NATURAL GAS HYDROGEN CORPORATION, OF NEW YORK, N. Y., A CORPORATION OF DELAWARE

## PROCESS OF RE-FORMING NATURAL GAS

Application filed July 8, 1930. Serial No. 466,559.

- It is not uncommon in cities in the natural gas districts that the supply of natural gas available is insufficient to meet the demand at all times. Under such circumstances it is necessary to provide an auxiliary supply of manufactured gas which may be mixed with the available natural gas to make up a sufficient bulk of gas to meet the peak demand. Also under some circumstances it is necessary or desirable to supply a consumer with a gas of lower calorific value than pure natural gas which may be done also by blending a manufactured gas of relatively lower calorific value with the natural gas.
- The gas to be blended with the natural gas may be producer gas, blue water gas, carburetted water gas or some other type of gas, for instance a gas made by the decomposition or partial combustion of the natural gas itself and it is customary for natural gas distributors to maintain a plant for the manufacture of artificial gas to supplement the natural gas supply or modify it to meet the demands of the consumer. Such a plant, as will be apparent, normally may be idle a large portion of the time and its cost of maintainence is therefore very high as compared with the quantity of gas produced by it.
- In supplementing a natural gas supply with manufactured gas and particularly when the amount of manufactured gas added to the natural gas varies, the character of the manufactured gas is quite important i. e. it is essential that the resulting blended gas shall not have burning characteristics so different from the normal gas supply as to cause the gas burning equipment of the consumer of the gas to function improperly.
- Factors to be considered in this connection are the specific gravity and flame propagation rate of the manufactured gas. In general a hydrogen content in the manufactured gas, due to its low specific gravity and high flame propagation rate is of value because these characteristics offset the effect of heavy inert gases and slow burning relatively heavy hydrocarbons, for example producer gas or carburetted agents which are frequently also introduced into the blended gas in order to provide the necessary bulk and/or calorific value.
- An object of the present invention is to provide a process which meets the above mentioned requirements. The process of my invention is capable of being carried out in certain types of the customary supplementary gas manufacturing equipment with only minor and relatively inexpensive modification, which apparatus may therefore be used part of the time in carrying out my process and at other times, if desired, for the manufacture of the particular kind of artificial gas for which it was designed. My process may serve to convert the natural gas into a manufactured gas of up to approximately double the volume of the natural gas which manufactured gas is capable of use as fuel directly or for blending with natural gas and thus may itself under circumstances quite frequently encountered serve to provide the excess volume of gas necessary to meet the peak demand. It yields a gas of high hydrogen content which is admirably suited for blending purposes and also a substantial amount of salable carbon black which materially offsets the cost of operation. At times when the process is not called upon for supplementing the normal natural gas supply and an excess of natural gas is available it may be operated to produce carbon black or industrial hydrogen or both or to produce combustible gas having special characteristics for certain industrial requirements and carbon black as a by-product. From the foregoing it will be seen that due to the flexibility of the process it is admirably adapted to the varied conditions and requirements of the gas utility business in ad-

dition to producing a blendable gas, which due to its high hydrogen content is admirably suited for blending purposes, and carbon black as a by-product so that the net 5 cost of the gas produced is less than for gas or similar quality made by the heretofore used methods.

The accompanying drawing is a dia-  
grammatic illustration in front elevation of  
10 one arrangement of apparatus suitable for  
carrying out the process.

Referring to the drawing 1 represents a standard water gas generator provided with inlets 2 and 3 for the introduction of gas, 15 steam and air into the generator, above and below the fuel bed and outlets 4 and 5 for the removal of gaseous products carrying carbon black in suspension for the generator above and below the fuel bed. For sim-  
plicity, the actual construction of the apparatus which is well known and the piping and valves for the introduction of air, gas and steam and the withdrawal of gaseous products which readily can be provided are 20 not illustrated. Pipes 4 and 5 deliver into a common conduit 6 through which the gases may flow to the stack 7 or to the carbon black recovery and gas purifying and storage apparatus 8, 9, 10, 11 and 12. It will  
25 be understood that the invention is not limited to the use of a conventional water gas generator but may employ an especially designed apparatus in which a fuel bed of coke of the desired size can be established  
30 and maintained and provided with means for the introduction and withdrawal of gases. It is further to be understood that the invention is not limited to any particular method of or apparatus for the treat-  
35 ment of the gases leaving the generator for the recovery of carbon black, the apparatus illustrated and described herein being merely one form of apparatus suitable for carrying  
40 out the process of the invention.

45 The conduit 6 delivers into a cooler 8 (which might be replaced by heat exchang-  
ing apparatus) in which the gases are sprayed with water to cool them to a temperature suitable for the subsequent treatment, say  
50 to about 400° F. The gases then pass through the electrostatic precipitator 9 and the cyclone device 10 both of conventional design, then through the oil scrubber 11 and the water scrubber 12 to storage,  
55 utilization or waste.

A typical procedure is as follows:

Using a nine foot generator with a fuel bed 8 feet deep, air is blasted for 3 minutes, the blast gases being wasted during the first  
60 2 1/4 minutes and saved during the last 3/4 minute. The fuel bed of coke is then sub-  
jected to a short steam purge, for instance about 1/2 minute, the resulting water gas being saved after which a gas run of about  
65 1000 cubic feet per minute for about 10 min-

utes is made, the resulting gases being saved. All of the gases passed through the fuel bed or only the gases produced during the gas run or only those saved may be passed through the apparatus 8, 9, 10, 11 and 12 70 for the recovery of carbon black and puri-  
fication of the gases. The mixture of the gases saved from the air blasting, the steam purge and the natural gas run, has a spe-  
cific gravity and heat value substantially 75 equal to that of blue water gas, and when the cost of the natural gas is within suit-  
able economic limits, this gas mixture is less expensive than blue water gas due largely 80 to the value of the carbon black recovered. In a specific instance requiring the admix-  
ture of equal parts of the manufactured gas and natural gas to produce a 550 B. t. u. gas, it was found possible to reduce the cost 85 of the resultant gas 50% as compared with  
gas of equal heat value prepared by blending natural gas with blue water gas. The proc-  
ess is subject to great variation depending upon various conditions which affect the results obtained and the specific object 90 sought. The type and size of the generator, composition of the natural gas, composition of the gas desired, kind and yield of carbon black desired, and kind of coke available may necessitate certain modifications of pro-  
cedure such as the thickness of the fuel bed, the size of the coke and the rate and 95 periods of running on air, steam and natural gas. To produce a gas of high heat value, e. g., by limiting the cracking of the hydrocarbon, the period of contact of the gas with the fuel bed may be limited by 100 passing the gas at a rapid rate, or using a thinner fuel bed, or both, or by running the gas for a longer period, or with the fuel bed at a lower temperature, whereas to 105 produce a gas of high hydrogen content and low heat value the conditions generally are reversed, i. e., the conditions are adjusted so as to afford a relatively long contact be-  
tween the gas and the coke at a high tem-  
perature. Generally a temperature above 1200° C. or in the range 1200 to 1400° C. is employed. To maintain the fuel bed con-  
tinuously at optimum operating condition, 110 the air and gas runs may be reversed from time to time or periodically or split, that is part of the run may be in one direction and the remainder of the run in the oppo-  
site direction through the fuel bed. It is also desirable occasionally or periodically, 115 say every fourth or fifth run to substitute for a gas run a steam run generally of shorter duration, to condition the fuel bed. The steam run seems to clear the fuel bed of deposited carbon and to prevent caking. In any event a steam run generally results in a reduction of the resistance of the fuel bed to the flow of gas through it, as well 125 as a reduction in coke consumption. The 130

steam purge serves to clear the producer of unconsumed air and thus to avoid explosions upon the introduction of gas.

A possible variation of the above described procedure is to introduce steam into the generator along with the natural gas thereby producing directly a combination of water gas and cracked natural gas suitable for use as fuel or for blending purposes.

Under certain circumstances a supply of so-called refinery gases, which are mixtures of hydrocarbons, carbon oxides, nitrogen, etc., resulting from the refining or cracking of petroleum, are available for utility use. These gases are quite similar in chemical composition and can be treated in the same manner for the production of a gas of high hydrogen content and carbon black, as a by-product, as natural gas. Such gases normally are of high heat value and specific gravity, both of which may be reduced to correspond with that of natural gas or of a manufactured gas with which they are to be blended or for which they are to be substituted.

In the appended claim natural gas embraces refinery gases and other gases of similar composition, i. e., consisting essentially of gaseous hydrocarbons as equivalents.

I claim:

Process of re-forming natural gas which comprises blasting a bed of coke at a temperature of about 1200° C., with air for about three minutes, to raise its temperature to about 1400° C., wasting the gases produced during about the first  $2\frac{1}{4}$  minutes of said 3 minute period and saving the gases produced during about the last  $\frac{3}{4}$  minute of said 3 minute period, purging the bed of coke with steam for about  $\frac{1}{2}$  minute, saving the resulting gases, and then passing natural gas through the bed of coke for about 8 to 10 minutes, saving the resulting gases, purifying the saved gases and recovering carbon black therefrom and mixing the purified gases for use as fuel, and continuously repeating the series of operations.

In testimony whereof, I affix my signature.

JAMES A. YUNKER.